

## UNITED STATES PATENT OFFICE

STAPLETON D. GOOCH, OF LAKE WALES, FLORIDA, ASSIGNOR TO CORONET PHOSPHATE COMPANY, OF NEW YORK, N. Y., A CORPORATION OF NEW YORK

## TREATMENT OF PHOSPHATIC MATERIAL

No Drawing.

Application filed March 4, 1930. Serial No. 433,185.

This invention relates to the treatment of phosphatic material.

In the ordinary method of preparing raw phosphatic material for the manufacture of 5 fertilizer, the material from the mine is screened or sized and then sent to a log washer to remove adherent sand, clay, and soft phosphate from the hard pebble. Thereafter the rock is subjected to a further washing or 10 rinsing operation. After this treatment the rock is quite wet and in order to prepare it for subsequent treatment for the manufacture of fertilizer it must be dried.

The drying of the wet rock is usually done 15 by heating it in a rotary kiln. In the ordinary method crude oil is used as the fuel for the kiln. After this drying operation the material is then ready for shipment to the fertilizer plant.

20 An object of the present invention is to provide a novel method of drying wet phosphate rock.

Another object is to devise a method of 25 treating phosphatic raw material to appreciably increase the  $P_2O_5$ .

A further object is to devise a method of 30 drying wet phosphate rock by utilizing the materials eventually produced from the rock.

Yet another object is to devise a simple 35 method of increasing the availability of phosphate rock.

An additional object is to effect economy 40 in the preparation of phosphate fertilizer by subjecting wet phosphate rock to a preliminary treatment to dry the material and simultaneously to partially convert it to an available form.

With these and other equally important objects in view the invention comprehends the 45 concept of generating drying heats *in situ* in the wet rock and by means of a material which is a potentially available conversion re-agent for the rock.

To enable a ready comprehension of the 50 invention a preferred method will be herein-after described, but it will be understood that the treatment and material specified are merely illustrative and are to be considered 55 as indicative of the equivalent steps and sub-

stances which may be employed to effect the desired novel results.

In carrying out the invention wet phosphate rock is fed to the upper end of a rotary kiln and simultaneously therewith there is 60 fed a readily combustible substance, the heat of combustion of which is utilized to expel the water from the rock. The preferred pyrogenetic substance is elemental phosphorus. This material may be fed, either as 65 a sludge or as a substantially solid mass, into the kiln at a point adjacent the entrant position of the rock, or the streams of rock and phosphorus may be combined and the single or confluent stream then led directly to the 70 burner or kiln.

It will be appreciated that the method and place of admission of the two materials, as 75 well as the particular mechanisms utilized, may be widely varied. Thus the materials 80 may be conveyed to the inlet end of the drier by a belt or screw conveyors or by any other suitable means. These are mechanical arrangements which may be varied as desired to adapt and accommodate the present process 85 to any particular existing equipment.

Simultaneously with the admission of the rock and phosphorus there is injected into the kiln a stream of air of sufficient volume to insure complete oxidation of the phosphorus. 90 This air may be admitted under natural or forced draft. In these circumstances, the phosphorus ignites and the heat of combustion generated, so to speak, *in situ* expels or drives off the moisture in the rock. Due to 95 the presence of water vapor and to the large contact surface afforded by the rock a certain amount of phosphoric acid is formed. The phosphoric acid so formed reacts with the tricalcium phosphate to form citrate soluble 100 phosphate. This simple treatment, therefore, effects two desirable results; it dries the wet phosphate and simultaneously increases the  $P_2O_5$  content of the rock. This increase in  $P_2O_5$  content is additionally advantageous 105 because of the fact that it is largely in an available form. This material, therefore, presents an excellent raw material for subsequent treatment with acid in the manufacture of phosphate fertilizers. Inasmuch as it con-

tains a large percentage of available phosphate less acid is required in making up super or double super phosphates or any fertilizer mixtures.

5 The excess  $P_2O_5$  formed by the combustion of the phosphorus passes out of the drier, at the discharge end, and is then admitted to a suitable absorption system wherein it is sprayed with phosphoric acid or to a Cottrell precipitator wherein it is collected as strong phosphoric acid, or if desired, it may be passed through both of these systems in series.

10 It will be observed that the present method at once provides a process for drying phosphate and/or enriching phosphate. The water necessary for the humidification of the  $P_2O_5$  may be derived either from water contained in the rock or from water used as a vehicle for the elemental phosphorus. Therefore, the method is applicable to substantially dry phosphate rock for the purpose of increasing its  $P_2O_5$  content. In such a treatment the water necessary for the production of phosphoric acid is furnished by the aqueous vehicle of the elemental phosphorus. Furthermore, it is observed that the drying of the phosphate rock is more effectively carried out due to the fact that the heat of oxidation of the phosphorus is generated, so to speak, *in situ*, that is to say, directly in contact with and uniformly disseminated through the mass.

15 It is to be observed that the process is susceptible of many variations and ramifications. For example, if it is desired to increase the  $P_2O_5$  content to the optimum degree, the rock may be finely divided before admitting it to the drier. It is to be observed here that since the process is applicable to wet 20 rock the economies derived from wet grinding may be obtained. With a fine subdivision of the rock a greater reactive surface is presented and a consequent increase in the quantity of the reaction products is secured. This reaction 25 may, of course, be increased by supplementing the action of the phosphoric acid formed in the drier with that admitted to the drier from the absorption tower or Cottrell precipitator.

30 While the process has been described as involving the utilization of elemental phosphorus it is to be understood that it is not necessarily limited to this material. The concept of drying wet phosphate rock by heats generated in the body of the rock may be 35 effectuated by using other oxidizable materials. Elemental phosphorus is preferred for a number of reasons. In the first place, it enables the system to be, so to speak, self-contained. In lieu of using fuel oil as a means of deriving drying heats, elemental phosphorus obtained by the pyrolysis under reducing conditions of a phosphate silica mixture 40 may be employed. In this manner the product of one of the units (an electric or fuel

45 furnace) of a plant may be utilized as the fuel and as the potentially available re-agent for the treatment described, so as to obtain a relatively concentrated product which will withstand heavy freight charges. The process 50 also increases the possibility of utilizing low or medium grade phosphate deposits which, due to their relatively low phosphate content, are unfit for treatment with sulphuric acid.

55 It is to be understood, however, that the invention is not limited to the use of a material such as phosphorus which subserves all of the improved functions described herein. Other materials which will oxidize and whose heat of oxidation may be utilized to dry wet phosphate rock may be employed. Such materials as will accomplish any or all of the described functions and results are considered as being comprehended within the spirit of the invention.

I claim:

1. The method of drying moist phosphatic material comprising mixing phosphorus with the material and then burning the phosphorus in contact with the material, while maintaining the temperature below that at which phosphorus in the phosphate rock is reduced and volatilized.

2. The method of drying and enriching phosphate rock comprising burning free phosphorus in contact with the rock and maintaining the temperature below that at which phosphorus in phosphate rock would be reduced and volatilized.

3. The method of drying phosphate rock comprising simultaneously feeding the rock and elemental phosphorus to a rotary burner and effecting combustion of the phosphorus therein.

4. The method of drying and increasing the  $P_2O_5$  content of phosphate rock comprising simultaneously feeding moist phosphate rock and phosphorus into a combustion zone, causing combustion of the phosphorus therein in direct contact with the rock to thereby utilize the heat of combustion of the phosphorus to dry the rock and absorbing at least a part of the phosphoric acid produced in the rock and thereby effect a partial conversion of unavailable phosphatic material to an available form.

5. The method of drying and enriching moist phosphatic material comprising adding elemental phosphorus to the moist material generating  $P_2O_5$  *in situ* in the material to thereby utilize the heat of combustion of the phosphorus to dry the material, forming phosphoric acid therefrom in contact with and from moisture derived from the material.

6. The method of enriching and drying wet phosphate rock comprising simultaneously feeding rock and elemental phosphorus to a rotary burner agitating the mixture in said burner causing combustion of the phos-

phorus therein, absorbing some of the  $P_2O_5$  by the rock, and utilizing the heat of combustion of the phosphorus to expel moisture from the rock.

5 7. The method of treating wet phosphate rock comprising simultaneously passing elemental phosphorus and the rock to a rotary burner, causing combination of the phosphorus, agitating and contacting the rock with the products of combustion to increase the  $P_2O_5$  content and discharging and collecting the excess  $P_2O_5$ .

10 8. A method of drying moist phosphatic material comprising subjecting the material to exothermic heat generated in situ by the formation of phosphorus pentoxide from the oxidation of free added phosphorus, and maintaining the temperatures sufficiently low to prevent the reduction and volatilization of phosphorus in the phosphatic material, but sufficiently high to expel excess water and to convert at least a portion of the phosphatic material to citrate soluble phosphate.

15 9. A method of enriching and drying moist phosphate rock comprising generating phosphorus pentoxide directly in contact with the phosphate rock by the combustion of added elemental phosphorus and humidifying the phosphorus pentoxide generated with water derived from the moist rock, thereby utilizing the heat of combustion of the phosphorus to expel water from the rock and to cause a conversion of a portion of the rock to citrate soluble phosphate.

20 35 In testimony whereof I affix my signature.  
STAPLETON D. GOOCH.

40

45

50

55

60

65